

# UNITED STATES PATENT OFFICE.

WILLIAM C. PEASE, OF MARIETTA, OHIO.

## COPPER ALLOY.

1,168,962.

Specification of Letters Patent.

Patented Jan. 18, 1916.

No Drawing.

Application filed January 25, 1915. Serial No. 4,356.

*To all whom it may concern:*

Be it known that I, WILLIAM C. PEASE, a citizen of the United States, residing at Marietta, in the county of Washington and State of Ohio, have invented certain new and useful Improvements in Copper Alloys, of which the following is a specification.

This invention comprehends certain new and useful improvements in the art of metallurgy and relates particularly to a novel process of tempering or hardening copper, and to a new and useful metal or alloy produced thereby.

As is well known to those versed in the art to which this invention appertains, pure copper is soft and not capable of being worked up into tools, bearings, and the like, and with a knowledge of these conditions, my invention has for its primary object a simple and efficient process whereby the required temper and hardness may be secured so that the product formed by the carrying out of the process hereinafter described will constitute a metal that will take and maintain an edge, and that may be subjected to considerable friction and abrasive action without becoming appreciably or unduly worn, and will also be applicable in different arts where a non-corrosive and relatively hard metal may be required.

With these and other objects in view as will more fully appear as the description proceeds, the invention consists in the various steps employed, in the ingredients used, and the manner in which they are combined and in the metal or alloy itself in its completed condition, all as will be hereinafter more fully described and claimed.

For a full understanding of the invention, reference is to be had to the following description, in which I shall first describe the method used in producing the metal, then describe the completed article or metal from an analytical standpoint, and finally conclude with the claims wherein I shall set forth what I consider to be new with me.

In carrying out my invention, I take aluminium and iron pyrites in the ore; I melt the aluminium in a crucible and while it is melting add a small piece of clay of any of the ordinary kinds about the size of a hen's egg for each pound of aluminium. When this mass has been thoroughly melted, I add the iron pyrites and after the melted mass with the pyrites therein has been stirred well, I pour it off into any suitable form and

after it has hardened it is broken up preferably in small pieces.

The copper to be hardened is weighed and is put in a crucible and melted in the usual manner. When it has been melted, I add one ounce of the compound above described to each pound of the copper. I mix well by stirring and pour out into molds. The hardness can be varied by adding more or less of the compound and it is to be further noted that I may vary the proportions of the aluminium and the iron pyrites, according to the hardness desired. Ordinarily, for all usual purposes, I employ in the compound above described, sixteen parts of aluminium to two parts of iron pyrites, but as above stated, that ratio is not always adhered to, but may be varied at will. The hardness of the metal or alloy can be still further increased by remelting the copper hardened in the manner hereinbefore described, and then adding a predetermined quantity of antimony, but it is to be understood that my invention is not limited to the use of antimony, although the use thereof possesses advantages under certain conditions, as is manifest.

By carrying out the process hereinbefore described, I produce a metal which has much the appearance of bronze or gold, and which possesses the requisite hardness to render it susceptible of being applicable for use in various arts, the metal being capable of being molded, machined, or forged into any desired shape and into any desired articles.

Preferably, the metal or alloy in its completed form comprises the following chemical substances, and preferably in the following proportions, although as hereinbefore indicated, I want it to be understood that the proportions need not be adhered to and, in fact, some of the ingredients, as for example, antimony, may be entirely dispensed with, according to the particular requirements of the case.

When antimony constitutes one of the substances or ingredients which together, in combined form, go to make up the tempered or hardened copper, the following substances are used and preferably in the following proportions, namely: copper, 88.4; aluminium, 6.6; antimony, 1.26; iron, 1.96; silicon, 1.60.

When antimony is not used, the remaining ingredients are preferably in the following proportions, although it is to be

understood that these proportions need not be adhered to, namely: copper, 94.13; silicon, .74; aluminium, 3.08; iron, 1.80.

Having now described my improved metal or alloy, and the manner in which it is preferably produced, what I claim as new, is:

1. The herein described alloy of copper, consisting of the following ingredients in substantially the following proportions, copper, 88.4 oz., aluminium, 6.6 oz., antimony, 1.26 oz., iron, 1.96 oz., and silicon, 1.60 oz.

2. An alloy of copper containing the following ingredients in substantially the following proportions, namely, 88.4 per cent. of copper; 6.6 per cent. of aluminium; 1.96 per cent. of iron; and 1.60 per cent. of silicon.

In testimony whereof I affix my signature in presence of two witnesses.

WILLIAM C. PEASE.

Witnesses:

D. W. GALL,  
FREDERICK S. STITT.